

## 1

3,751,406

### AZO COMPOUNDS USEFUL IN PHOTOGRAPHIC PROCESSES

Stanley M. Bloom, Waban, Mass., assignor to Polaroid Corporation, Cambridge, Mass.

No Drawing. Filed July 24, 1967, Ser. No. 655,338  
Int. Cl. C07c 107/04, 107/06, 107/08

U.S. Cl. 260—162 17 Claims

#### ABSTRACT OF THE DISCLOSURE

Compounds which are useful in photographic processes for producing colored image patterns. The compounds initially are immobile and non-diffusible in photographic processing compositions. However, when oxidized, the compounds undergo intermolecular rearrangement to split off a mobile and diffusible color providing material.

#### BACKGROUND OF THE INVENTION

The copending application of Stanley M. Bloom and Howard G. Rogers, Serial No. 655,440, now U.S. Pats. 3,443,940, filed concurrently, relates to novel photographic systems for preparing color images. In these systems, a photosensitive element including at least one light-sensitive silver halide emulsion is developed in the presence of a compound which is immobile and non-diffusible in the processing fluid, but which, upon development, undergoes a ring-closing reaction to split off a mobile and diffusible color-providing material. Color image formation is predicated upon the resulting differential in diffusibility, whereby an imagewise distribution of the more diffusible color-providing material split off as a function of development may be transferred to an image-receiving layer, e.g., a dyeable stratum of the character heretofore known in the art, to provide a color transfer image thereon.

The present invention relates to novel compounds which may be employed in the various photographic products and processes described and claimed in this copending application.

#### SUMMARY

These compounds may be defined as being compounds which are immobile and non-diffusible in an aqueous alkaline processing medium and which are capable of reacting with an oxidized silver halide developing agent of the type known as "color developers" or which are capable of providing an oxidation product which may auto-react intramolecularly in such a way as to form a new heterocyclic ring, and as a function of such reaction and ring formation to split off a mobile and diffusible color-providing material.

They may also be defined as being within one of the following groups of compounds:

(1) Relatively immobile and non-diffusible compounds capable of coupling with the oxidation product of an aromatic primary amino color developer during development of an exposed silver halide emulsion with subsequent ring closure to produce a new heterocyclic ring and as a function of such reaction to split off a mobile and diffusible color-providing material; or

(2) Relatively immobile and non-diffusible silver halide developing agents which are capable of providing, upon development of an exposed silver halide emulsion, an oxidation product which can auto-react intramolecularly to

## 2

form a new heterocyclic ring and as a function of such reaction to split off a mobile and diffusible color-providing material.

As was mentioned previously, this invention is directed to novel compounds including a color-providing moiety and which are of particular use in the photographic systems described and claimed in the aforementioned copending application Ser. No. 655,440, now U.S. Pat. 3,443,940.

10 A primary object of this invention, therefore, is to provide a novel class of compounds of the foregoing description and methods for preparing the same.

Another object is to provide a novel class of compounds which are particularly useful in color photography.

15 Other objects of the invention will in part be obvious and will in part appear hereinafter.

The invention accordingly comprises the product possessing the features, properties and the relation of components which are exemplified in the following detailed disclosure.

20 For a fuller understanding of the nature and objects of the invention, reference should be had to the following detailed description.

The novel compounds of this invention may be represented by the following formula:

(A)



wherein:

35 A represents the atoms necessary to complete an aromatic ring, e.g., a benzene or naphthalene nucleus, which nucleus may be further substituted;

D is a color-providing moiety, e.g., a complete dye such as a monoazo, disazo, or anthraquinone dye, which may, if desired, be metallized in known manner;

40 Z may be hydrogen, any of the substituents heretofore known in the art which are replaceable by oxidized aromatic amino color developer in so-called elimination-coupling reactions (see, for example, Mees, "The Theory of the Photographic Process," Revised Edition, 1954, pp. 599-601), e.g., chloro, bromo, carboxy, sulfo, hydroxy, alkoxy, hydroxyalkyl, etc.; or an aromatic amino radical, e.g., an anilino substituent, including substituted anilino radicals, particularly of the p-hydroxyanilino series or the substituted anilino radical of a color developer of the p-phenylene diamine series, e.g.,



55 wherein:

Each R<sup>2</sup> is hydrogen or a lower alkyl radical, and including the known substituted derivatives of the aforementioned anilino radicals having a free position ortho to the —NH— substituent, a para-amino or a para-hydroxy-naphthylamino radical, including substituted derivatives thereof having a free position ortho to the —NH— substituent, which derivatives may contain an anchoring moiety to be described with more particularity hereinafter;

Y is any substituent which completes or forms an amide with, and reduces the basic character of the amino group in the 3-position, such as the residue of an acid, linking the color-providing moiety D to the 3-nitrogen atom, and which is capable of being eliminated during the ring formation to be described with more particularity herein-after, e.g.,



etc.;

X is hydroxy or amino, e.g., a primary, secondary or tertiary amino substituent of the formula:



wherein:

Each R<sup>3</sup> may be hydrogen, a hydrocarbon radical, e.g., alkyl, such as methyl, ethyl, butyl, dodecyl, etc., aryl such as phenyl or naphthyl attached through a carbon atom thereof to the nitrogen atom, a cyclic alkyl such as cyclopentyl or cyclohexyl, i.e., where both R<sup>3</sup>'s are alkylene comprising together with the nitrogen atom a heterocyclic ring, a substituted alkyl, such as hydroxyethyl, methoxyethoxyethyl, polyglycoloxyethyl, carboxymethyl, carboxyethyl, ethyl-carboxymethyl, benzyl, phenylethyl, sulfo-phenylethyl, acetylaminophenylethyl, succinylaminophenylethyl, furanemethyl, etc.; or a substituted aryl such as methylphenyl, ethylphenyl, etc.; or when Z is one of the described anilino or naphthylamino radicals containing a para-amino or para-hydroxy substituent, X may be hydrogen or the substituent R;

R is an "anchoring" or immobilizing substituent rendering the compound non-diffusible, e.g., higher alkyl such as decyl, dodecyl, stearyl, oleyl, etc. linked directly to the aromatic nucleus or linked indirectly thereto through an appropriate linking group, e.g., —CONH—,



etc., an aromatic ring, e.g., of the benzene or naphthalene series, or a heterocyclic ring, which rings may be either bonded to a single carbon atom of the aromatic nucleus or fused thereto, i.e., bonded to a pair of adjacent carbon atoms, or R may be a plurality of short chain radicals which together provide the anchoring moiety, each of said short chain radicals being linked directly or indirectly to a different carbon atom of the aromatic nucleus formed by the A moiety;

R<sup>1</sup> is hydrogen, an alkyl such as methyl, ethyl, propyl, butyl, hexyl, octyl, dodecyl, cyclohexyl, etc.; or a substituted alkyl, e.g., a hydroxyalkyl, such as 2-hydroxyethyl, 3-dihydroxypropyl, etc., carboxyalkyl such as carboxymethyl, carboxyethyl, carboxybutyl, carboxydecyl, etc., hydroxyethyl-ether, polyglycoloxyethyl, furanemethyl, benzyl, phenylethyl, carboxyphenylethyl, sulfo-phenylethyl, acylamino-phenylethyl, etc.;

And n is a positive integer from 1 to 2, provided that when R<sup>1</sup> or R<sup>3</sup> alone or together comprise one of those named substituents rendering the compound non-diffusible, i.e., an "anchoring" substituent, and/or when Z comprises an aromatic nucleus contributing an anchoring moiety alone or in conjunction with said R<sup>1</sup> and/or R<sup>3</sup> moieties, n may be 1, but when R<sup>1</sup>, R<sup>3</sup> or Z alone or together do not provide such a substituent, n must be 2.

The various substituents described above which may provide the R, R<sup>1</sup>, R<sup>2</sup>, R<sup>3</sup>, Z and/or Y moieties and illus-

trative compounds containing the same are disclosed, for example, in one or more of the following U.S. Pats.: 2,414,491; 2,486,440; 2,522,802; 2,536,010; 2,543,338; 3,227,550; 3,227,551; 3,227,552; 3,227,554; 3,243,294; and 3,245,795.

As was mentioned previously, Z may be a substituted anilino radical of a color developer of the p-phenylene diamines series. As examples of color developers of this series which may contribute the aforementioned radical, mention may be made of the following:

N,N-diethyl-p-phenylenediamine,  
2-amino-5-diethylamino toluene,  
N-ethyl-β-methanesulfonamido-ethyl-3-methyl-4-amino-aniline,

15 4-amino-N-ethyl-3-methyl-N-(β-sulfoethyl)aniline,  
4-amino-N-ethyl-3-methoxy-N-(β-sulfoethyl)aniline,

4-amino-N-ethyl-N-(β-hydroxyethyl)aniline,  
4-amino-N,N-diethyl-3-hydroxymethyl aniline,

4-amino-N-methyl-N-(β-carboxyethyl)aniline,  
4-amino-N,N-bis(β-hydroxyethyl)aniline,

4-amino-N,N-bis(β-hydroxyethyl)-3-methyl aniline,  
3-acetamido-4-amino-N,N-bis(β-hydroxyethyl)aniline,  
4-amino-N-ethyl-N-(2,3-dihydroxypropyl)-3-methyl aniline sulfate salt

25 4-amino-N,N-diethyl-3-(3-hydroxypropoxy)aniline,  
and the like.

Also as was mentioned previously, the color-providing moiety D is not restricted to complete dyes and is intended to include within its scope materials which are initially colorless or of a color other than that ultimately desired in a particular environment, but which provide the desired color during or subsequent to use in the aforementioned photographic procedures, e.g., upon a change in environment and/or upon subsequent chemical reaction. This change of environment may, for example, be a change in pH, e.g., to an acid environment. Color-providing materials of this nature include indicator dyes, leuco dyes and carbonyls of basic dyes. Also included within the scope of this invention are incomplete dyes or color formers which may react with another substance to form a dye image. However, an incomplete dye or a color former of this description must not be reactable with the oxidized color developer so as to preclude ring-closure and release of the diffusible color-providing moiety.

In general, compounds within the scope of Formula A may be readily synthesized by appropriate reaction between an acid salt of the desired dye and the 3-amino substituent of the aromatic ring, as follows:



Where X is amino, it may be necessary or desirable 70 to employ the corresponding 1-nitro analogues in the aforementioned reaction, followed by reduction, e.g., with hydrogen in the presence of a Raney nickel catalyst, to form a 1-amino compound within the scope of Formula A. It may also be desirable, in some instances, to have the 1-amino substituent protected during reaction, e.g.,

by an appropriate blocking group, to insure reaction between the acid salt and the 3-amino substituent.

As examples of useful compounds within the scope of Formula B, mention may be made of the following:

(1)



The compounds wherein Z is a coupling position may be represented by the following formula:

(B)



(2)



15

(3)



20

25

(4)



30

35



(6)



(7)



(8)



The compounds of Formula A wherein Z is an aromatic amino substituent may be represented by the following formula:

(C)



wherein:

X<sup>2</sup> is hydrogen, hydroxy, an amino group of the formula:



such as may be contained by said X moiety, as previously described, or the substituent R<sup>4</sup>, provided that at least one of said X and X<sup>2</sup> moieties must be hydroxy or amino;

A<sup>1</sup> represents the atoms necessary to complete a benzene or naphthalene ring, which ring may be further substituted:

R<sup>4</sup> has the same meaning as R;

n<sup>1</sup>, like n is a positive integer from 1 to 2, provided that when R<sup>1</sup> or R<sup>3</sup> alone or together comprise one of those heretofore named substituents rendering the compound non-diffusible, either or both n and n<sup>1</sup> may be 1, but when R<sup>1</sup> and R<sup>3</sup> alone or together do not provide such an anchoring moiety, at least one of n and n<sup>1</sup> must be 2.

The compounds of Formula C may be prepared by coupling a dye of the formula:

(D) Cl—Y—D

with a compound of the formula:

(E)



Where X and/or X<sup>2</sup> is hydroxy, it may be necessary or advisable for the hydroxy moiety to be present as a protected derivative, e.g., as an alkoxy substituent, during coupling, in which event the desired hydroxy analogue may subsequently be obtained by hydrolysis.

The preferred compounds of Formula C may be represented by the formula:

(F)



wherein the anchoring moiety R or R<sup>4</sup> comprises a long chain amide, e.g., of at least 13 carbon atoms, said amide being bonded directly to a nuclear carbon atom of the designated benzene moiety or being linked thereto through a phenylene or alkylene linking substituent; and nuclear substituted derivatives thereof, e.g., where any of the nuclear carbon atoms of the respective benzene moieties not containing one of the specifically designated substituents may contain a carboxy, alkyl, alkoxy, amino, chloro, hydroxyl, or amide substituent, etc.

The preferred subclass of Formula F may be prepared by coupling in the manner described with regard to the broader class of Formula C followed by dealkylation of the protected hydroxy group. Where the starting materials are not readily available, they may be prepared by the steps set forth in the following sequence of reaction steps:



They may also be prepared by coupling of any of the protected derivatives of the known p-aminophenol developers, with an ortho-fluoro-nitrobenzene, followed by reduction of the nitro group, coupling of the dye-containing moiety D—SO<sub>2</sub>—Cl, and hydrolysis in the aforementioned manner, according to the procedure described and claimed in the copending application of Harris L. Curtis, Ser. No. 655,304 filed July 24, 1967 filed concurrently.

As examples of useful compounds contemplated by Formula C mention may be made of the following:

(9)



(10)



(11)



(12)



(13)



(14)

5

10

15

25

30

35

40

45

50

60

65

70

75



11



12



(27)



(28)



(29)



(30)



(31)



Compounds 24 and 25 contain a color-shifted yellow dye moiety; and Compounds 28, 29, and 31 contain a color-shifted magenta dye moiety. These compounds are initially substantially colorless but upon hydrolysis, e.g., in an alkaline photographic processing fluid, provide the desired color. Color-shifted yellow dyes and magenta dyes and their advantages in photography are described with more particularity in U.S. Pats. No. 3,230,085 and 3,307,947, respectively.

The following examples show by way of illustration and not by way of limitation the preparation of the novel compounds of this invention.

## 14 EXAMPLE 1

500 g. of methyl p-amino-benzoate were added to 1,250 ml. of acetic anhydride with stirring, while maintaining the temperature of the mixture between 50° and 60° C.

5 After addition was complete, the mixture was chilled. A white solid, which precipitated, was removed by suction filtration and air-dried under a hood. 509.7 g. (79.8%) of 4-carbo-methoxyacetanilide (M.P. 131–133° C.) were obtained. A mixture of 315.8 g. of (1.63 moles) of this 10 compound, 1,250 ml. of glacial acetic acid, and 600 ml. of acetic anhydride was stirred with external cooling until the temperature dropped to about 2° C. Nitrous fumes, prepared from 500 g. of sodium nitrite and 500 ml. of nitric acid (sp. gr. 1.42), were bubbled into the mixture 15 for two hours, after which time the resulting dark green, clear solution was stirred into 5 l. of crushed ice. A light yellow precipitate was removed by suction filtration, washed thoroughly with water, pressed between filter papers, and then dried in vacuo over anhydrous calcium 20 chloride to yield 250.2 g. (68.8%) of 4-carbo-methoxy-N-nitroacetanilide. Over a period of two hours with vigorous stirring, 250.2 g. (1.13 moles) of this compound were added to 560 g. (2.98 moles) of molten 4-chloro-3-nitroanisole. The temperature of the mixture was kept 25 between 50° and 60° C. during the addition. Stirring was continued for an additional 15 minutes, after which the excess anisole was removed by steam distillation. The resulting dark brown residue was triturated with 1,500 ml. of ether. The ether-insoluble solid was removed by 30 suction filtration and washed with small portions of ether. One recrystallization of this solid from ethanol yielded 18.5 g. (5.8%) of (2-methoxy-4-nitro-5-chloro-4'-carbo-methoxy)diphenyl, M.P. 189–191° C., having the following structural formula:

35



45 To a 14.2 g. (0.466 m.) of this compound in 400 ml. of methylene chloride, 75 ml. of boron tribromide were 50 carefully added. The resulting dark red solution was allowed to stand overnight at room temperature and then treated dropwise with anhydrous methanol until further 55 addition of methanol no longer produced an exothermic reaction. After treatment with water, the mixture was extracted with ether, the ether layer extracted with cold 1% sodium hydroxide solution, the alkaline solution was filtered and acidified with hydrochloric acid. The resulting cream-colored solid was filtered, washed with water and dried. 12 g. of (2-hydroxy-4-nitro-5-chloro-4'-carbo-methoxy)diphenyl were obtained. [This product was 60 found to contain free acid, N.P. soft 238° C., M. 250–253° C. dec. A small amount of ester was purified by extraction with sodium bicarbonate solution followed by recrystallization from methanol, M.P. 235–237° C.] A mixture of 12 g. of the diphenyl prepared above, 250 ml. of ethanol and 75 ml. of 10% sodium hydroxide solution was heated on the steam bath for 30 minutes. The resulting red solution was filtered, acidified with hydrochloric acid, filtered, washed and dried to yield 11.4 g. of (2-hydroxy-4-nitro-5-chloro-4'-carbo-methoxy)diphenyl, M.P. 251–252° C. 4 g. of this compound, 40 ml. of acetic anhydride and 1 ml. of pyridine were heated on a steam bath 65 for five hours. The resulting solution was evaporated to dryness and the residue recrystallized from ethyl acetate-hexane to yield 4.5 g. of (2-acetoxy-4-nitro-5-chloro-4'-carbo-methoxy)diphenyl, M.P. 211.5–213.5° C. A mixture of 4.5 g. of this compound and thionyl chloride was refluxed 70 for one hour. The excess thionyl chloride was then allowed to stand overnight. The resulting solution was 75

15

lowed to distill at atmospheric pressure over 30 minutes and the residue was evaporated at 40° C. at water-pump pressure. The yellow solid acid chloride was directly dissolved in 250 ml. of dry benzene and added dropwise with stirring to a solution of 6 g. of dodecylamine hydrochloride in 25 ml. of triethylamine at ice bath temperature. The mixture was allowed to stir overnight at room temperature, after which it was poured into dilute hydrochloric acid solution and extracted with methylene chloride. The organic layer was washed three times with dilute hydrochloric acid solution, then with water until the aqueous layer was neutral to pH paper. The methylene chloride solution was dried over anhydrous magnesium sulfate, filtered and evaporated to dryness to yield a brown oil. The brown oil was chromatographed on Florisil using ether-hexane and the product was present in the first yellow band which eluted. Partial evaporation of the ether solvent and addition of hexane produced waxy yellow flakes. A recrystallization from ether-hexane and another from methylene chloride-carbon tetrachloride produced 2.8 g. (in two crops) of (2-hydroxy-4-nitro-5-chloro-4'-carbo-n-dodecylamide)diphenyl, M.P. 145-148° C., having the following structural formula:



A mixture of 2.76 g. of this compound, 150 ml. of anhydrous ethanol, 1 ml. of concentrated hydrochloric acid and about 2 g. of 5% palladium on carbon was hydrogenated at room temperature at an initial pressure of 40 lbs. per square inch. Reduction required about one hour. The mixture was then filtered, the residue washed with anhydrous ethanol and the filtrate evaporated to a low volume. Anhydrous ether was added to the colorless solution and upon cooling, 2.7 g. of (2-hydroxy-4-amino-hydrochloride - 5 - chloro-4'-carbo - n - dodecylamide)diphenyl was obtained, M.P. 207-215° C. dec. A mixture of 1 g. of this compound and 1.4 g. of 4-(2-naphthol-1-azo) benzene sulfonyl chloride in 50 ml. of pyridine was stirred at room temperature for three hours at which time complete solution was obtained. The solution was allowed to stand at room temperature overnight, poured into ice-water and filtered. After work-up of the mother liquor and recrystallization from glacial acetic acid, 1.2 g. of the compound of Formula 1 was obtained, M.P. 229-232° C.  $\lambda_{\text{max.}} = 482$ ;  $\epsilon = 23,400$  in methyl Cellosolve.

#### EXAMPLE 2

11.0 g. (0.05 mole) of 6-nitrodehydrocoumarin was dissolved in 100.0 cc. of methyl Cellosolve. 12.0 g. (0.064 mole) of n-dodecylamine was then added. [The reaction was exothermic and a yellow solid separated out.] The mixture was heated until a clear solution was obtained and then cooled to give 14.0 g. of light yellow crystals, M.P. 168-170, an amide of the formula:



A mixture of 16.5 g. (0.0437 mole) of this amide, prepared in the manner described above, 7.0 g. (0.056 mole) of dimethylsulfate, 9.2 g. (0.066 mole) of potassium carbonate and 250 ml. of xylene was refluxed overnight. The xylene was then removed by steam distillation and an oily product crystallized on standing. Recrystallization of this

16

product from hexane-chloroform yielded 13.3 g. of light tan needles, M.P. 106-108° C. of the formula:



10 13.3 g. of this latter amide was hydrogenated in 95% ethanol in the presence of a Raney-Nickel catalyst. The reaction mixture was filtered and the filtrate evaporated. The resulting solid was recrystallized from hexane-ether to obtain 9 g. of a pure white amine, M.P. 80-82° C. of the formula:



25 52 g. (0.145 mole) of the amine prepared in the above manner, 21.0 g. (0.145 mole) of 2-fluoronitrobenzene, 7.85 g. (0.195 mole) of magnesium oxide and 100.0 ml. of water were heated in a sealed bomb at 180° C. for 18 hours. The contents of the bomb were then filtered and the solid obtained by filtering was stirred in boiling ethyl acetate and filtered. Cooling of the filtrate yielded 40 g. of a light yellow solid, M.P. 125-126° C., of the formula:



40 45 10.0 g. of the last-named product was hydrogenated with 5% Pd/BaSO<sub>4</sub> in ethyl acetate to reduce the nitro group to the corresponding amine. The reaction mixture was filtered and the filtrate was then cooled in Dry Ice. Filtration yielded 9 g. of an off-white solid, M.P. 81-83° C., of an amine of the formula:



60 65 4.54 g. (0.01 mole) of this amine and 3.5 g. (0.1 mole) of the sulfonyl chloride of Orange II, a dye of the formula:



were allowed to stand overnight at room temperature in 100 ml. of pyridine. The reaction mixture was then heated

17

on the steam bath for 30 minutes, allowed to cool and poured into 500 ml. of 10% HCl and 50 g. of ice. The resulting solid was filtered and recrystallized from ethyl acetate-methanol to yield 3.6 g. of an orange solid, M.P. 191-123° C. of the formula:



2.6 g. (0.0034 mole) of this solid in 50 ml. of methylene chloride was reacted with a large excess of boron tribromide in methylene chloride and the reaction mixture was allowed to stand at room temperature overnight. Water was cautiously added and when the reaction was complete, the mixture was stirred for one hour while bubbling nitrogen through the solution. The resulting orange solid was collected by filtration and crystallized from 25 methanol to yield 2.6 g. of the compound, M.P. 150-151° C. of Formula 19.

## EXAMPLE 3

The procedure of Example 2 was repeated, substituting 30  $n\text{-C}_{18}\text{H}_{37}\text{NH}_2$  for the dodecylamine to obtain the compound of Formula 20.

## EXAMPLE 4

15 g. of sodium carbonate was dissolved in 500 ml. of 35 water. 57.3 g. of sulfanilic acid monohydrate was then slowly added. After all of this acid was dissolved, the resulting solution was cooled to 0° C. and 22.5 g. of sodium nitrite was added. After the sodium nitrite had dissolved, the resulting solution was poured into a mixture of 40 60.0 ml. of 37% HCl and 300 g. of ice to form a diazonium salt of the formula:



After formation of this diazonium salt, the reaction mixture was poured into a water-acetone solution of 15.9 g. of sodium carbonate and 69.6 g. of:



The resulting mixture was allowed to stand for several hours, and then filtered to yield 125 g. of:



To a stirred slurry of 20 g. of this last-named compound in 50 ml. of water, was added 20.0 ml. of *n*-propylamine. The resulting mixture was refluxed with stirring overnight. Excess propylamine was boiled off and the remaining mixture was poured into 20% NaCl. After filtra-

18

tion and recrystallization, 15.5 g. of the corresponding amide was obtained, M.P. 272-274° C. of the formula:



10.4 g. of this amide, 50.0 ml. of chlorobenzene, 5.0 ml. of thionyl chloride and 4.0 ml. of *N,N*-dimethylformamide where heated on a steam bath for one hour.

15 The solvent was then removed by evaporation with a stream of nitrogen and the resulting mixture was triturated with hexane-benzene. Filtration and recrystallization from benzene yielded 4 g. of a compound, M.P. 185-187° C. of the formula:



3.4 g. of this compound and 3.4 g. of an amine of the formula:



(prepared in the manner described in Example 2) were 45 refluxed overnight in 50 ml. of dry benzene. The mixture was then cooled and the resulting solid collected and crystallized from benzene to yield 4 g. of a compound, M.P. 133-135° C. of the formula:



65 4.0 g. of this last-named compound in 50 ml. of dichloromethane was reacted with a large excess of boron tribromide and the reaction mixture was then allowed to stand overnight at room temperature. Water was added to

70 "destroy" excess boron tribromide and the mixture was then stirred under nitrogen for one hour and filtered. The resulting solid residue was stirred in hot water and filtered. Recrystallization from benzene-hexane yielded 2.0 g. of the compound of Formula 21, yellow crystals, 75 M.P. 138-140° C.

19  
EXAMPLE 5

Fifteen grams of 4-fluoro-5-nitro-aniline, 35.0 grams of stearoyl chloride and 8.4 g. of sodium bicarbonate were stirred overnight at room temperature. The reaction mixture was then refluxed and the insoluble inorganic salts were filtered off. Upon cooling of the filtrate, an off-white solid was obtained, M.P. 82-83° C., having the formula:



Thirty grams of 3-carboxy-4-methoxy-aniline was added to 75.0 g. of the 5-stearamido-2-fluoro-nitrobenzene (prepared above) and 45.0 g. of potassium acetate in 225 ml. of dimethyl sulfoxide. The resulting mixture was stirred over a weekend under a flow of nitrogen while maintaining the temperature at about 100° C. It was then poured into a large amount of cold water and the resulting precipitate was filtered, washed with water and a small amount of ethanol. This crude product was then recrystallized from acetic acid to yield 36 g. of a yellow solid, M.P. 186-187° C., of the formula:



Four grams of the last-mentioned compound was hydrogenated in ethanol with a Pd/BaSO<sub>4</sub> catalyst to reduce the nitro group to an amino substituent. Following hydrogenation for about two hours, the product was filtered and quickly cooled to obtain 3 g. of the amine, a nearly white solid, M.P. 115° C. Seven g. of this amine was added to 4.7 g. of 4'-(sulfonyl-chloride)-phenylazo-2-naphthol in 100 ml. of pyridine under nitrogen. The mixture was allowed to stand overnight at room temperature. It was then heated on a steam cone for 30 minutes, then poured into 600 ml. of 10% HCl, filtered and then rinsed with water and a small amount of methanol. The resulting solid was next triturated with warm methylene chloride and filtered to yield 4.6 g. of a yellow solid, M.P. 138-140° C., of the formula:



5.0 g. of the last-named compound was added to an unmeasured amount (about 60 ml.) of methylene chloride and 15 ml. of boron tribromide. The mixture was stirred overnight. The starting material went into solution as it complexed with the boron tribromide. The complex was decomposed with water, then triturated with hot water, methanol and hexane to yield 4.6 g. of the compound of Formula 16, a yellow solid, M.P. 260° C.

The following examples illustrate the use of the compounds of this invention in the photographic systems described and claimed in the aforementioned application Ser. No. 655,440, now U.S. Pat. 3,443,940.

20  
EXAMPLE 6

5 A first coating solution was prepared containing a mixture of 0.14 g. of the compound of Formula 1, 0.2 g. of cellulose acetate hydrogen phthalate, 5.0 cc. of acetone and 7.0 cc. of methyl Cellosolve. This solution was coated at room temperature at a rate of 10 feet per minute on a cellulose triacetate base which had been coated with 200 mg. per square foot of gelatin. After this coating had dried, a second coating solution was applied at the same rate containing 8.0 cc. of a standard light-sensitive silver iodobromide emulsion, 28.0 cc. of water, and 2.0 cc. of 1% aqueous "Triton X-100" (trademark for a nonionic isoctyl phenyl polyethoxy ethanol dispersing agent). This coating was made in the dark with the temperature of the coating solution kept at 40° C. The resulting photosensitive element was exposed for  $\frac{1}{100}$  of a second and the thus exposed element was then developed by spreading between this element and a superposed image-receiving element at a gap of .0036", a processing composition comprising the following proportions of ingredients:

10 Water ----- cc. 100.0  
Hydroxyethyl cellulose ----- g. 3.9  
Potassium hydroxide ----- g. 4.9  
25 ADAT (2 - amino - 5 - N,N - diethylamino-  
toluene) ----- g. 2.0

30 The image-receiving element was prepared in accordance with the disclosure of the copending application of Edwin H. Land, Ser. No. 234,864, filed Nov. 1, 1962 and comprised a layer of a 2:1 mixture by weight of polyvinyl alcohol and poly-4-vinyl pyridine, a layer of polyvinyl alcohol, and a layer of a half-butyl ester of poly(ethylene/maleic anhydride) coated on a baryta paper support. After an imbibition period of about three minutes, the image-receiving element was separated to reveal thereon a negative yellow-orange image.

## EXAMPLE 7

40 Five cc. of a dispersion containing a 10:20:11 ratio, by weight, of the compound of Formula 19, N,N-diethyl decanamide and gelatin, was mixed with 13 cc. of water, 5 cc. of a colloidal silver silver-precipitating agent mixture containing .08 g. of Ag/100 cc. of water, 2 cc. of 1% aqueous "Triton X-100" (trademark for a nonionic isoctyl phenyl polyethoxy ethanol dispersing agent), and 1 cc. of 5% aqueous ethanol. The resulting mixture was coated on a cellulose acetate support at 10 feet per minute at 40° C. After this coating had dried, a mixture of 4 cc. of a blue-sensitive silver iodobromide emulsion, 32 cc. of water and 2 cc. of 1% "Triton X-100" was coated thereover at the same speed and temperature to provide a photosensitive element.

55 The efficacy of a system using a photosensitive element prepared in the foregoing manner was first established by typical testing procedures wherein the ability of the color-providing material to transfer from unexposed areas was confirmed. In such testing procedures, no attempt is made to obtain an image and the unexposed element is imbibed with a processing composition containing no developer while in superposition with a dyeable stratum.

60 This unexposed element was imbibed with an aqueous alkaline processing composition containing no silver halide developer to establish that transfer could be effected in terms of unexposed areas. This was ascertained by spreading between the unexposed element and a superposed dyeable stratum at a gap of .0024" a composition comprising the following proportions of ingredients:

65 Water ----- cc. 100.0  
Hydroxyethyl cellulose ----- g. 3.9  
Sodium hydroxide ----- g. 5.0  
70 Sodium thiosulfate ----- g. 4.0

75 Following an imbibition period of about two minutes, the respective elements were separated to reveal a uniform dense orange dye transfer image.

## EXAMPLE 8

A photosensitive element similar to that prepared in the above example was prepared by coating onto a cellulose acetate support at a rate of 10 feet per minute a mixture containing 10 cc. of 2% cellulose acetate hydrogen phthalate in acetone, 3.5 cc. of the aqueous colloidal silver mixture in cellulose diacetate and 1.5 g. of the compound of Formula 19; and thereafter coating onto the thus formed layer at the same rate a mixture containing 4.0 cc. of a panchromatic silver halide emulsion, 24.0 cc. of water and 1.0 cc. of 2% "Aerosol O.T." (trademark for a wetting agent, dioctyl sodium sulfosuccinate). This photosensitive element was exposed and then developed by spreading between the thus exposed element and a superposed dyeable sheet material at a gap of .0024" a processing composition containing the following proportions of ingredients:

|                        |     |       |
|------------------------|-----|-------|
| Water                  | cc. | 100.0 |
| Hydroxyethyl cellulose | g.  | 3.9   |
| Sodium hydroxide       | g.  | 5.0   |
| Sodium thiosulfate     | g.  | 2.0   |
| Triptycene diol        | g.  | 1.0   |

After an imbibition period of about two minutes, the elements were separated to reveal a positive dye image.

The compounds of Formulae (C) and (F), e.g., the illustrative Compounds 9-31, may also be employed in the photographic systems described and claimed in the copending applications of Stanley M. Bloom and Robert K. Stephens, Ser. Nos. 655,501, filed July 24, 1967 and 655,436, filed July 24, 1967, both filed concurrently.

They may also be employed in the manner in which dyes have heretofore been employed, e.g., in the dyeing of fabrics, etc.

Since certain changes may be made in the above product without departing from the scope of the invention herein involved, it is intended that all matter contained in the above description shall be interpreted as illustrative and not in a limiting sense.

What is claimed is:

1. A compound of the formula:



wherein:

A represents the atoms necessary to complete a benzene or naphthalene radical;

D is a monoazo or disazo dye;

Z is hydrogen, a substituent replaceable by oxidized aromatic amino color developer in elimination-coupling reactions, said substituent being selected from the group consisting of chloro, bromo, carboxy, sulfo, hydroxy, alkoxy and hydroxylalkyl or Z may be the residue of an oxidized aromatic amino color developer;

Y is the residue of an acid forming an amide with and reducing the basic character of the nitrogen atom to which it is bonded and is selected from the group consisting of



X is hydroxy, a primary, secondary or tertiary amino of the formula



wherein each R<sup>3</sup> is hydrogen, alkyl, phenyl, naphthyl, or each R<sup>3</sup> may be alkylene so that the R<sup>3</sup>'s together with the nitrogen atom provide a heterocyclic ring having 5 or 6 carbon atoms or each R<sup>3</sup> may be a lower alkyl having a substituent chosen from the group consisting of a hydroxy substituent, a methoxyethoxy substituent, a polyglycoloxy substituent, a carboxy substituent, an ethoxycarboxy substituent, a benzyl substituent, a phenyl substituent, a sulfo-phenyl substituent, an acetylaminophenyl substituent, a succinylaminophenyl substituent or a furane substituent or when Z is the residue of an oxidized amino color developer containing a p-amino or p-hydroxy substituent, X may be hydrogen or the substituent R;

5 15 R is an anchoring substituent rendering the compound non-diffusible, said substituent containing a higher alkyl radical bonded to a single carbon atom of said aromatic nucleus formed by said A moiety;

R<sup>1</sup> is hydrogen or alkyl; and

20 n is 1 or 2 provided that n may be 1 when X is a secondary or tertiary amino comprising an anchoring moiety rendering said compound non-diffusible or when R<sup>1</sup> is an alkyl radical providing an anchoring moiety or when Z comprises the residue of an oxidized aromatic amino color developer and said residue contributes an anchoring moiety, but when R<sup>1</sup>, X or Z do not provide such an anchoring moiety, n must be 2.

25 2. A compound as defined in claim 1 wherein X is hydroxy or a primary, secondary or tertiary amino of the formula



30 35 wherein each R<sup>3</sup> is hydrogen, alkyl, phenyl, naphthyl or each R<sup>3</sup> may be alkylene so that the R<sup>3</sup>'s together with the nitrogen atom provide a heterocyclic ring having 5 or 6 carbon atoms or each R<sup>3</sup> may be a lower alkyl having a substituent chosen from the group consisting of a hydroxy substituent, a methoxyethoxy substituent, a polyglycoloxy substituent, a carboxy substituent, an ethoxycarboxy substituent, a benzyl substituent, a phenyl substituent, a sulfo-phenyl substituent, an acetylaminophenyl substituent, a succinylaminophenyl substituent or a furane substituent.

40 45 3. A compound as defined in claim 1 wherein R comprises a higher alkyl linked directly to said aromatic nucleus or indirectly through a —CONH—,



50 or



55 substituent.

4. A compound of the formula



60 65 wherein:

A represents the atoms necessary to complete a benzene or naphthalene radical;

D is a monoazo or disazo dye moiety;

Z<sup>1</sup> is hydrogen or a substituent replaceable by an oxidized aromatic amino color developer in elimination-coupling reactions, said substituent being selected from the group consisting of chloro, bromo, carboxy, sulfo, hydroxy, alkoxy and hydroxylalkyl;

70 75 Y is the residue of an acid forming an amide with and reducing the basic character of the nitrogen atom to

which it is bonded and is selected from the group consisting of



$X^1$  is hydroxy or a primary, secondary or tertiary amino of the formula



wherein each  $R^3$  is hydrogen, alkyl, phenyl, naphthyl, or each  $R^3$  may be alkylene so that the  $R^3$ 's together with the nitrogen atom provide a heterocyclic ring having 5 or 6 carbon atoms or each  $R^3$  may be a lower alkyl having a substituent chosen from the group consisting of a hydroxy substituent, a methoxyethoxy substituent, a polyglycoloxyl substituent, a carboxy substituent, an ethoxycarboxy substituent, a benzyl substituent, a phenyl substituent, a sulfo-phenyl substituent, an acetylaminophenyl substituent, a succinylaminophenyl substituent or a furane substituent provided that at least one of  $X$  and  $X^2$  must be hydroxy or amino;

$R$  is an anchoring substituent rendering the compound non diffusible said substituent containing a higher alkyl radical bonded to a single carbon atom of said aromatic nucleus formed by said  $A$  moiety;

$R^1$  is hydrogen or alkyl; and

$n$  is 2 or  $n$  may be 1 when  $X^1$  is a secondary or tertiary amino comprising an anchoring moiety rendering said compound non diffusible or  $R^1$  is an alkyl radical providing such an anchoring moiety.

5. A compound as defined in claim 4 wherein  $R^1$  is hydrogen, and  $n$  is 2.

6. A compound as defined in claim 4 wherein  $R$  comprises a higher alkyl linked directly to said aromatic nucleus or indirectly through a  $\text{CONH}$ —



or



substituent.

7. A compound of the formula



wherein:

each of  $A$  and  $A^1$  represents the atoms necessary to complete a benzene or naphthalene radical;

$D$  is a monoazo or disazo dye moiety;

$Y$  is the residue of an acid forming an amide with and reducing the basic character of the nitrogen atom to which it is bonded and is selected from the group consisting of



$X$  and  $X^2$  each is the substituent  $R$ , hydrogen, hydroxy, 70 a primary, secondary or tertiary amino of the formula



wherein each  $R^3$  is hydrogen, alkyl, phenyl, naphthyl, or each  $R^3$  may be alkylene so that the  $R^3$ 's together with the nitrogen atom provide a heterocyclic ring having 5 or 6 carbon atoms or each  $R^3$  may be a lower alkyl having a substituent chosen from the group consisting of a hydroxy substituent, a methoxyethoxy substituent, a polyglycoloxyl substituent, a carboxy substituent, an ethoxycarboxy substituent, a benzyl substituent, a phenyl substituent, a sulfo-phenyl substituent, an acetylaminophenyl substituent, a succinylaminophenyl substituent or a furane substituent provided that at least one of  $X$  and  $X^2$  must be hydroxy or amino;

$R$  and  $R^4$  each represent an anchoring substituent rendering the compound non diffusible, said substituent containing a higher alkyl radical bonded to a single carbon atom of said aromatic nucleus formed by said  $A$  or  $A^1$  moieties respectively;

15  $R^1$  is hydrogen or alkyl; and  $n$  and  $n^1$  each is 1 or 2 and each  $n$  and  $n^1$  may be 1 when one  $X$  or  $X^2$  is the substituent  $R$  or a secondary or tertiary amino comprising an anchoring moiety rendering the compound non diffusible or when  $R^1$  is an alkyl substituent providing such an anchoring moiety but when said substituents do not contribute an anchoring moiety, at least one of  $n$  and  $n^1$  must be 2.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9

25

the shown benzene moiety by a linking group which is  
—alkylene—CONH—, —CONH— or



and  $n$  is 2.

11. A compound of the formula:



wherein:

D is a monoazo dye moiety;

R<sup>1</sup> is hydrogen;

one of X<sup>1</sup> or X<sup>2</sup> is hydroxy or amino and the other is hydrogen or the substituent R;

each R is an anchoring moiety rendering the compound nondiffusible and comprises a higher alkyl of at least 10 carbon atoms bonded to a nuclear carbon atom of the shown benzene moiety by a linking group which is 30  
—alkylene—CONH—, —CONH— or



and one of  $n$  and  $n^1$  is 2 and the other is 1 unless X<sup>1</sup> or X<sup>2</sup> is R, in which case both  $n$  and  $n^1$  are 1.

12. A compound as defined in claim 4 wherein R comprises a higher alkyl linked directly to said aromatic nucleus or indirectly through a —CONH—,



or



substituent.

13.



14.



15.

26



5



15

16.



20



25

17.



35

40

45

50

55

#### References Cited

#### FOREIGN PATENTS

60 74,309 6/1952 Denmark ----- 260—197

LEWIS GOTTS, Primary Examiner

C. F. WARREN, Assistant Examiner

65 U.S. CL. X.R.

96—91, 29; 260—147, 152, 163, 174, 177, 178, 180, 181, 184, 185, 187, 188, 194, 195, 196, 197, 199, 201, 202, 203, 207, 207.1, 372, 373, 471 R, 519, 559 R, 559 A, 561 R

70